

## UNITED STATES PATENT OFFICE

2,369,449

## PRINT-OUT EMULSIONS

George E. Fallesen, Rochester, N. Y., assignor to  
 Eastman Kodak Company, Rochester, N. Y., a  
 corporation of New Jersey

No Drawing. Application December 14, 1943,  
 Serial No. 514,283

5 Claims. (Cl. 95—7)

This invention relates to photographic material and more particularly to a photographic emulsion of the type known as print-out emulsions.

Print-out emulsions are characterized by the fact that a visible image is produced in them directly by the action of light whereas developing emulsions or developing out emulsions must be subjected to the action of a developer in order to produce a visible image. The present invention relates to print-out emulsions and especially to those in which the light-sensitive element is a silver halide.

Print-out emulsions are usually prepared by the precipitation in a colloidal medium of a halide of silver by interaction of a solution of a soluble halide with a solution of a soluble compound of silver. In the case of print-out emulsions of silver chloride, the silver chloride is usually precipitated in the colloidal medium in such a way that the final product contains an excess of soluble silver compound, for instance, silver nitrate, the silver salt of an organic acid, such as silver citrate or silver tartrate, together with some of the free organic acid. The emulsions are not washed after precipitation of the silver halide. Print-out emulsions of silver bromide are prepared similarly.

The sensitivity to light of print-out emulsions may be increased by the addition of halogen absorbers such as soluble nitrates, alkaline materials such as borax, sodium hydroxide, ammonium hydroxide and organic alkalies such as pyridine or amines.

It is an object of the present invention to provide a different type of print-out emulsion. A further object is to provide a means for preparing a very fast print-out emulsion.

These objects are accomplished, according to my invention, by preparing a gelatino-silver halide emulsion containing an excess of soluble halide and adding to the emulsion thus prepared an appreciable amount of thiosalicylic acid. The emulsion used is preferably a moderately fast negative bromoiodide or pure bromide emulsion. The addition of thiosalicylic acid to such emulsion converts it into a very fast print-out emulsion.

A typical print-out emulsion, according to my invention, was prepared in the following manner:

A solution of 388 grams of silver nitrate in 3600 cc. of water, heated to 60° C., was mixed with a solution of 311 grams of potassium bromide in 2600 cc. of 1.8% gelatin solution, heated to 60° C. The silver nitrate solution was run into the bro-

5 mide gelatin solution in 30 minutes with stirring and the silver bromide was precipitated in the gelatin with an excess of potassium bromide. After the precipitation of the silver bromide, 215 grams of dry gelatin were added to the emulsion. A solution of 10 grams of thiosalicylic acid dissolved in 600 cc. of methyl-alcohol and adjusted with ammonium hydroxide to a pH of 6.9 was then added. The emulsion was heated for 30 minutes at 60° C. and was then chilled to set.

10 To finish the emulsion and prepare it for coating, it was washed, melted at 45° C., and 100 grams of gelatin were added to it at 70° C. to finish. The emulsion was then ready for coating.

15 The emulsion thus prepared was coated on a suitable support and dried. It was then exposed for 5 minutes on a print-out sensitometer through a power of 2 step tablet by a 500 watt lamp 24 inches from the material. The neutral density step tablet used for this exposure produced 12 steps on the material whereas a similar exposure of a commercial print-out material produced only 7 steps. This means that the print-out material produced according to my invention was 32 times 20 as fast as the commercial print-out material with 25 which it was compared.

20 The color of the densities produced upon exposure was neutral blue-gray and the color of the emulsion before exposure was yellowish-white or cream-white, depending upon whether potassium iodide had been used in the emulsion formula.

25 The amount of thiosalicylic acid used in the example above was 1 gram of thiosalicylic acid to about 43 grams of silver bromide. The preferred amount of thiosalicylic acid is, therefore, about 2% of the amount of silver halide in the emulsion. However, more or less than this amount can be employed and the thiosalicylic acid concentration may vary from about 20 mg. to 4000 mg. per 50 grams of silver halide.

30 It is to be understood that the examples and modifications included herein are illustrative only and that my invention is to be taken as limited only by the scope of the appended claims.

I claim:

35 1. The process of producing a light-sensitive print-out emulsion, which comprises precipitating a light-sensitive silver halide in gelatin to form an emulsion having an excess of soluble halide, and adding to the resulting emulsion from 20 to 4000 milligrams per 50 grams of silver halide of thiosalicylic acid.

40 2. The process of producing a light-sensitive print-out emulsion, which comprises precipitat-

ing a light-sensitive silver halide in gelatin to form an emulsion having an excess of soluble halide, and adding to the resulting emulsion approximately 2% by weight of the silver halide of thiosalicylic acid.

3. The process of producing a light-sensitive print-out emulsion, which comprises precipitating in gelatin a light-sensitive silver bromide to form an emulsion having an excess of soluble bromide, and then adding to the emulsion an amount of thiosalicylic acid which is approximately 2% by weight of the silver bromide.

4. A light-sensitive print-out emulsion comprising a gelatino-silver halide emulsion containing an excess of soluble bromide and from 20 to 4000 milligrams per 50 grams of silver halide of thiosalicylic acid.

5. A light-sensitive print-out emulsion comprising a gelatino-silver bromide emulsion containing an excess of soluble bromide and an amount of thiosalicylic acid which is approximately 2% by weight of the silver bromide.

GEORGE E. FALLESEN.